

## UNITED STATES PATENT OFFICE

2,204,620

## LUBRICATING COMPOSITION

Carl F. Prutton, Cleveland, and Albert K. Smith, Shaker Heights, Ohio, assignors, by mesne assignments, to The Lubri-Zol Development Corporation, Cleveland, Ohio, a corporation of Ohio

No Drawing. Original application July 26, 1934, Serial No. 737,070. Divided and this application October 22, 1937, Serial No. 170,500

2 Claims. (Cl. 87—9)

As disclosed in the application of Carl F. Prutton Serial No. 635,701, filed September 30, 1932, certain desirable improvements in the lubricating properties of lubricating oils may be secured by the combination therewith of certain halogenated additions, particularly halogenated or more specifically chlorinated carbon ring compounds.

We have discovered that certain oxygen bearing or containing halogenated organic compounds used independently or in combination with any suitable oil base produce a lubricating composition equal to, and in certain respects superior to, the results secured by the addition of halogenated carbon ring compounds to a suitable oil base. The lubricating composition according to our invention is particularly applicable for use as an extreme pressure lubricant.

For the definition of extreme pressure lubrication and the distinction thereof over low pressure or thick film lubrication, reference may be had to the specification of the above mentioned application.

It is among the objects of our invention, therefore, to provide a lubricating composition which shall be superior to any which has heretofore been available.

Other objects of our invention will appear as the description proceeds.

To the accomplishment of the foregoing and related ends, said invention, then, consists of the means hereinafter fully described and particularly pointed out in the claims, the following description setting forth in detail one approved combination of ingredients embodying our invention, such disclosed means constituting, however, but one of various forms in which the principle of the invention may be used.

Broadly stated, this invention comprises the use as lubricants of oxygen and halogen bearing or containing organic ring compounds used either independently or in combination with any suitable oil base such as pure mineral oil or an oil which contains sulphur in solution or in a stable form of colloidal suspension, either in uncombined form, or in the form of a sulphur compound.

We have found that oxygen and halogen bearing or containing carbon ring compounds have excellent lubricating properties when used alone and particularly for certain classes of uses.

We have also found that compounds of this type are capable of improving the lubricating properties of lubricating oils when added thereto even in relatively small amounts and particularly when such oil is employed for "thin film" or "extreme pressure" lubricating purposes. 5

We have also found that certain oxygen and halogen bearing or containing derivatives of organic ring compounds of the heterogeneous ring type, i. e., compounds in which atoms other than carbon are included in the ring structure may likewise be used as lubricants or additions to lubricating oils. 10

The addition of these oxygen and halogen bearing or containing organic ring compounds to a suitable oil base have been found to improve 15 the properties thereof to an even greater extent than certain similar halogenated hydrocarbons, notably when added in very small amounts.

The oxygen and halogen containing or bearing organic ring compounds, above referred to 20 may be classified as follows, viz:

I. "Carbon ring" type compounds

(a) Of the aromatic, or allied type, including derivatives of benzene, naphthalene, anthracene, 25 etc., also compounds of the bridged ring type, such as the terpenes, and related compounds.

(b) Of the class including the cycloparaffins, cyclo-olefines, etc. Examples of this class are 30 derivatives of the following:

(1) Hydrogenation products of benzene (e. g., cyclohexane, cyclohexene, cyclohexadiene).

(2) Hydrogenation products of naphthalene (e. g. decahydronaphthalene, tetrahydro- 35 naphthalene etc.)

(3) Naphthenes, naphthenic acid, etc.

(c) Of mixed type such as derivatives of indene, hydridene, hydranthracene, etc.

II. "Heterogeneous ring" type compounds 40

(a) Of the aromatic or allied type including derivatives of pyridine, quinoline, etc.

(b) Other types such as furan and its derivatives and derivatives of thiophene, pyrrole etc. 45

The foregoing compounds may also be classified according to the nature of the attachment of the oxygen to the compound, viz:

I. Directly attached to one or more carbon atoms, as in the case of:

|    |                                                                                                                                                                                                                                                                                                                                                              | Halogen derivatives of— Class                     |    |
|----|--------------------------------------------------------------------------------------------------------------------------------------------------------------------------------------------------------------------------------------------------------------------------------------------------------------------------------------------------------------|---------------------------------------------------|----|
|    | (1') Ethers and analogous compounds                                                                                                                                                                                                                                                                                                                          | Benzyl naphthenate.I(b)-(3)-I'(3')                |    |
|    | (2') Compounds containing the $\equiv C-OH$ radicle, such as alcohols and other derivatives or carbinol (including phenols, cresols, naphthols etc.)                                                                                                                                                                                                         | Benzyl nitrate.I(a)-II'                           |    |
| 5  | (3') Compounds containing the carbonyl ( $=C=O$ ) radicle, such as aldehydes, ketones, organic acids, esters and salts of organic acids, thio-acids and esters of thio-acids                                                                                                                                                                                 | Benzyl nitrite.I(a)-II'                           |    |
| 10 | (4') Compounds in which oxygen forms a part of the ring structure, e. g., furan and its derivatives, anthraquinone, etc.                                                                                                                                                                                                                                     | Benzyl stearate.I(a)-I'(3')                       | 5  |
|    | II'. Indirectly attached through the means of some other atom, i. e., in the form of an inorganic radicle, e. g.:                                                                                                                                                                                                                                            | Benzyl sulphate.I(a)-II'                          |    |
| 15 |                                                                                                                                                                                                                                                                                                                                                              | Benzyl sulphite.I(a)-II'                          |    |
|    |                                                                                                                                                                                                                                                                                                                                                              | Benzyl sulphone.I(a)-II'                          |    |
|    |                                                                                                                                                                                                                                                                                                                                                              | Benzyl thio-sulphate.I(a)-II'                     |    |
| 20 | Amide                                                                                                                                                                                                                                                                                                                                                        | Pyrrole carboxylic acid.II(b)-I'(3')              | 10 |
|    | Arsenate                                                                                                                                                                                                                                                                                                                                                     | Thiophene carboxylic acid.II(b)-I'(3')            |    |
|    | Arsenite                                                                                                                                                                                                                                                                                                                                                     | Butyl benzoate.I(a)-I'(3')                        |    |
|    | Chlorate                                                                                                                                                                                                                                                                                                                                                     | Butyl thio-benzoate.I(a)-I'(3')                   | 20 |
|    | Chlorite                                                                                                                                                                                                                                                                                                                                                     | Butyl ester of mercapto rosolic acid.I(a)-I'(3')  |    |
|    | Cyanate                                                                                                                                                                                                                                                                                                                                                      | Butyl ester of phenyl acetic acid.I(a)-I'(3')     |    |
|    | Hydroxylamine                                                                                                                                                                                                                                                                                                                                                | Butyl ester of phenyl stearic acid.I(a)-I'(3')    | 25 |
|    | Hypochlorite                                                                                                                                                                                                                                                                                                                                                 | Butyl furoate.II(b)-I'(3') and (4')               |    |
| 25 | Nitrate                                                                                                                                                                                                                                                                                                                                                      | Butyl mercapto benzoate.I(a)-I'(3')               |    |
|    | Nitrite                                                                                                                                                                                                                                                                                                                                                      | Butyl naphthenate.I(a)-I'(3')                     | 30 |
|    | Nitro                                                                                                                                                                                                                                                                                                                                                        | Butyl phenyl ketone.I(a)-I'(3')                   |    |
|    | Nitroso                                                                                                                                                                                                                                                                                                                                                      | Butyl toluate.I(a)-I'(3')                         |    |
| 30 | In addition to the substituents containing oxygen, other substituents may also be present without destroying, and in certain cases improving, the effect on the lubricating qualities of the oil such as other aryl groups, alkyl groups, and amino and substituted amino groups, imino, azo, hydrazo, hydrazine, nitrile, mercapto, sulphide, polysulphide. | Calcium naphthenate.I(b)-I'(3')                   |    |
| 35 | Specific examples of compounds of the various classes described above are halogen derivatives of the compounds listed below. These derivatives may be substitution products, addition products, or both. They may be formed by halogenation of the compound listed, or of intermediate compounds, or by some other method.                                   | Calcium phenyl mercapto stearate.I(a)-I'(3')      | 35 |
| 40 | 45 Halogen derivatives of— Class                                                                                                                                                                                                                                                                                                                             | Calcium phenyl stearate.I(a)-I'(3')               |    |
|    | Acetanilide.I(a)-I'(3')                                                                                                                                                                                                                                                                                                                                      | Camphor.I(a)-I'(2')                               |    |
|    | Acetophenone.I(a)-I'(3')                                                                                                                                                                                                                                                                                                                                     | Cinnamic acid and esters.I(a)-I'(3')              | 40 |
|    | Aluminum phenyl mercaptostearate.I(a)-I'(3')                                                                                                                                                                                                                                                                                                                 | Cresyl acetate.I(a)-I'(3')                        |    |
| 50 | Aluminum phenyl stearate.I(a)-I'(3')                                                                                                                                                                                                                                                                                                                         | Cresyl naphthenate.I(b)-(3)-I'(3')                |    |
|    | Amyl salicylate.I(a)-I'(2') and (3')                                                                                                                                                                                                                                                                                                                         | Cresyl stearate.I(a)-I'(3')                       |    |
|    | Amino phenol.I(a)-I'(2')                                                                                                                                                                                                                                                                                                                                     | Cyclohexanol.I(b)-(1)-I'(2')                      | 45 |
|    | Anethole.I(a)-I'(3')                                                                                                                                                                                                                                                                                                                                         | Cyclohexanone.I(b)-(1)-I'(3')                     |    |
| 55 | Aniline oleate.I(a)-I'(2')                                                                                                                                                                                                                                                                                                                                   | Decahydronaphthol.I(b)-(2)-I'(2')                 |    |
|    | Aniline stearate.I(a)-I'(2')                                                                                                                                                                                                                                                                                                                                 | Dibenzoyldimethyl disulphide.I(a)-I'(3')          |    |
|    | Anthraquinone.I(c)-I'(2')                                                                                                                                                                                                                                                                                                                                    | Dibenzoyldimethyl sulphide.I(a)-I'(3')            | 50 |
|    | Anthranol.I(a)-I'(2')                                                                                                                                                                                                                                                                                                                                        | Dibenzoyl disulphide.I(a)-I'(3')                  |    |
|    | Azobenzoic acid.I(a)-I'(3')                                                                                                                                                                                                                                                                                                                                  | Dibenzoyl sulphide.I(a)-I'(3')                    |    |
| 60 | Azophenol.I(a)-I'(2')                                                                                                                                                                                                                                                                                                                                        | Dibenzyl ether.I(a)-I'(1')                        |    |
|    | Benzaldehyde.I(a)-I'(3')                                                                                                                                                                                                                                                                                                                                     | Di-butyl phthalate.I(a)-I'(3')                    |    |
|    | Benzaldoxime.I(a)-II'                                                                                                                                                                                                                                                                                                                                        | Di-disulphide of tertiary amyl phenol.I(a)-I'(2') |    |
|    | Benzamide.I(a)-II'                                                                                                                                                                                                                                                                                                                                           | Dihydroxy dibenzyl disulphide.I(a)-I'(2')         | 60 |
|    | Benzene sulphonic acid.I(a)-II'                                                                                                                                                                                                                                                                                                                              | Dihydroxy diphenyl disulphide.I(a)-I'(2')         |    |
| 65 | Benzene sulphoxide.I(a)-II'                                                                                                                                                                                                                                                                                                                                  | Dihydroxy diphenyl sulphide.I(a)-I'(2')           | 65 |
|    | Benzil.I(a)-I'(2')                                                                                                                                                                                                                                                                                                                                           | Dinaphthyl ether.I(a)-I'(1')                      |    |
|    | Benzoic acid.I(a)-I'(3')                                                                                                                                                                                                                                                                                                                                     | Dinaphthyl ketone.I(a)-I'(3')                     |    |
|    | Benzoin.I(a)-I'(2') and (3')                                                                                                                                                                                                                                                                                                                                 | Diphenyl acetic acid and esters.I(a)-I'(3')       |    |
| 70 | Benzophenone.I(a)-I'(3')                                                                                                                                                                                                                                                                                                                                     | Diphenyl ether.I(a)-I'(1')                        | 70 |
|    | Benzyl acetate.I(a)-I'(3')                                                                                                                                                                                                                                                                                                                                   | Dixenyl ether.I(a)-I'(1')                         |    |
|    | Benzyl alcohol.I(a)-I'(2')                                                                                                                                                                                                                                                                                                                                   | Ethyl ester of phenyl acetic acid.I(a)-I'(3')     |    |
|    | Benzyl cyanate.I(a)-II'                                                                                                                                                                                                                                                                                                                                      | Ether naphthyl ether.I(a)-I'(1')                  |    |
|    | Benzyl mercapto stearate.I(a)-I'(3')                                                                                                                                                                                                                                                                                                                         |                                                   | 75 |

| Halogen derivatives of— |                           | Class | Halogen derivatives of—          | Class          |
|-------------------------|---------------------------|-------|----------------------------------|----------------|
| Ethyl salicylic acid    |                           |       | Phenyl hydroxyl-                 |                |
| and esters              | I(a)-I'(2') and (3')      |       | amine                            | I(a)-II'       |
| Ethyl toluate           | I(a)-I'(3')               |       | Phenyl mercapto                  |                |
| Furan                   | II(b)-I'(4')              |       | stearate                         | I(a)-I'(3')    |
| Furfural                | II(b)-I'(3') and (4')     |       | Phenyl mercapto                  |                |
| Furil                   | II(b)-I'(3') and (4')     |       | stearic acid and                 |                |
| Furoin                  | II(b)-I'(2')(3') and (4') |       | esters                           | I(a)-I'(3')    |
| Hexahydrophenyl         |                           |       | Phenyl napthenate                | I(b)(3)-I'(3') |
| acetate                 | I(b)(1)-I'(3')            |       | Phenyl naphthyl                  |                |
| Hexahydrophenyl         |                           |       | ketone                           | I(a)-I'(3')    |
| mercapto stearate       | I(b)(1)-I'(3')            |       | Phenyl nitrite                   | I(a)-II'       |
| Hexahydrophenyl         |                           |       | Phenyl oleate                    | I(a)-I'(3')    |
| stearate                | I(b)(1)-I'(3')            |       | Phenyl oxydisul-                 |                |
| Hydroxyazobenzene       | I(a)-I'(2')               |       | phide                            | I(a)-I'(3')    |
| Hydroxy - b e n z y l   |                           |       | Phenyl phenol                    | I(a)-I'(2')    |
| mercaptan               | I(a)-I'(2')               |       | Phenylphenyl ace-                |                |
| Hydroxy - diphenyl-     |                           |       | ta te                            | I(a)-I'(3')    |
| amine                   | I(a)-I'(2)                |       | Phenylphenyl                     |                |
| Hydroxy-indene          | I(c)-I'(2)                |       | napthenate                       | I(b)(3)-I'(3') |
| Hydroxy - methyl -      |                           |       | Phenylphenyl                     |                |
| aniline                 | I(a)-I'(2)                |       | stearate                         | I(a)-I'(3')    |
| Hydroxy - phenyl -      |                           |       | Phenyl propionic                 |                |
| hydrazine               | I(a)-I'(2')               |       | acid and esters                  | I(a)-I'(3')    |
| Hydro x y p h e n y l   |                           |       | Phenyl propyl al-                |                |
| mercaptan               | I(a)-I'(2')               |       | cohol                            | I(a)-I'(2')    |
| Hydroxy-quinoline       | II(a)-I'(2')              |       | Phenyl stearate                  | I(a)-I'(3')    |
| Hydroxythiophene        | II(b)-I'(2')              |       | Phenyl stearic acid              | I(a)-I'(3')    |
| Iminophenol             | I(a)-I'(2)                |       | Pyridine stearate                | II(a)-I'(3')   |
| Indoxyl                 | I(c)(2)-I'(2)             |       | Pyrrol stearate                  | II(b)-I'(3')   |
| Ketopentam e th y l     |                           |       | Sodium phenylmer-                | I(a)-I'(3')    |
| ene                     | I(b)-I'(3')               |       | captostearate                    |                |
| Mercapto benzoic        |                           |       | Sodium phenyl - I(a)-I'(3')      |                |
| acid                    | I(a)-I'(3')               |       | stearate                         |                |
| Mercapto r o s o l i c  |                           |       | Sodium thioben- I(a)-I'(3')      |                |
| acid                    | I(a)-I'(3')               |       | zoate                            |                |
| Methyl salicylate       | I(a)-I'(2') and (3')      |       | Stearanilid                      | I(a)-I'(3')    |
| Methyl toluate          | I(a)-I'(3')               |       | Tertiary amyl phe- I(a)-(I')(2') |                |
| Naphthol                | I(a)-I'(2')               |       | nol                              |                |
| N a p h t o l e t h y l |                           |       | Thiobenzoic acid                 | I(a)-I'(3')    |
| ether                   | I(a)-I'                   |       | Toluic acid                      | I(a)-I'(3')    |
| Nitrodiphenyl           | I(a)-I'                   |       | Tricresyl phosphate              | I(a)-II'       |
| Nitrosobenzene          | I(a)-II'                  |       | Triphenyl arsenate               | I(a)-II'       |
| Nitrosophenol           | I(a)-II'                  |       | Triphenyl arsenite               | I(a)-II'       |
| Nitrotoluene            | I(a)-II'                  |       | Triphenyl phos - I(a)-II'        |                |
| Phenol                  | I(a)-I'(2')               |       | phate                            |                |
| Phenyl acetate          | I(a)-I'(3')               |       | Triphenyl phos - I(a)-II'        |                |
| Phenyl acetic acid      | I(a)-I'(3')               |       | phite                            |                |
| Phenyl amyl nitrate     | I(a)-II'                  |       | Tri-tertiary amyl - I(a)-II'     |                |
| Phenyl amyl nitrite     | I(a)-II'                  |       | phenyl phosphate                 |                |
| Phenyl amyl ether       | I(a)-I'(1')               |       | Zinc benzoate                    | I(a)-I'(3')    |
| Phenyl benzoate         | I(a)-I'(3')               |       | Zinc phenylstearate              | I(a)-I'(3')    |
| Phenyl ethyl al-        |                           |       |                                  |                |
| cohol                   | I(a)-I'(2')               |       |                                  |                |
| Phenyl ethyl chlo-      |                           |       |                                  |                |
| rate                    | I(a)-II'                  |       |                                  |                |
| Phenyl ethyl chlo-      |                           |       |                                  |                |
| rite                    | I(a)-II'                  |       |                                  |                |
| Phenyl ethyl cya-       |                           |       |                                  |                |
| inate                   | I(a)-II'                  |       |                                  |                |
| Phenyl ethyl ether      | I(a)-I'(1')               |       |                                  |                |
| Phenyl ethyl hypo-      |                           |       |                                  |                |
| chlorite                | I(a)-II'                  |       |                                  |                |
| Phenyl ethyl per-       |                           |       |                                  |                |
| chlorate                | I(a)-II'                  |       |                                  |                |
| Phenyl ethyl sul-       |                           |       |                                  |                |
| phate                   | I(a)-II'                  |       |                                  |                |
| Phenyl ethyl sul-       |                           |       |                                  |                |
| phite                   | I(a)-II'                  |       |                                  |                |
| Phenyl ethyl sul-       |                           |       |                                  |                |
| phone                   | I(a)-II'                  |       |                                  |                |
| Phenyl ethyl thio-      |                           |       |                                  |                |
| sulphate                | I(a)-II'                  |       |                                  |                |

One theory of the action of halogen compounds, specifically chlorine compounds, in increasing film strength assumes that, under the stress of the rubbing action of bearing surfaces in motion under load, chlorides of the bearing metals are formed on their surfaces and exert an "anti-fluxing" effect in preventing subsequent fusing of the two surfaces. This surface reaction, however, to take place with sufficient effectiveness depends upon the hydrolysis of the chlorine compound as a simultaneous intermediate reaction. These reactions may be expressed as:



where R is an organic radicle and M is one of 70 the metals of the bearing surfaces.

(Note.—The hydrogen evolved by (2) probably would act to reduce one or more of the organic compounds present rather than to appear as free hydrogen.)

This theory is substantiated by the fact that when a chlorinated hydrocarbon is added to a hydrocarbon mineral oil and the mixture is thoroughly freed from moisture by the action of dehydrating agents, the film strength is no more than that of the oil alone. Exposure of the mixture to the atmosphere, so that it may adsorb a slight amount of moisture, will then cause an increase in the film strength. Since the presence of a large amount of moisture, and especially of free water, is objectionable in a lubricant, besides being a highly variable factor in normal service, it is advisable to supply an oil-soluble substitute for it in the form of an organic oxygen compound. Even a small amount, say 0.1% or less of such a compound in combination with a chlorinated hydrocarbon (or other oxygen-free organic halogen compound) acts to increase the effectiveness of the latter in raising the film strength of a mineral oil, or to improve the lubricating properties of the chlorinated compound when used without the addition of some other lubricant. The organic oxygen compound probably acts in the same way as water in making possible the formation of HCl as an intermediate step by some such reaction as:



30 (Note.—Since atomic hydrogen is always available in one or both of the organic radicles, R and R', it need not be attached to the oxygen atom in the form of hydroxyl, as in this example.)

35 In the case of organic oxygen compounds which are very strongly adsorbed by metal surfaces, (e. g., fatty acids and derivatives of them) if too much is added, the chlorine compound may be prevented from functioning to increase the film strength, probably by being displaced from such surfaces. It is, therefore, advisable to determine the amount of the oxygen compound used which will have the optimum effect.

40 By combining in a single molecule the halogen and the oxygen atoms, still further improvement is effected in two ways: (1) the oxygen is always available at the exact point where required; and (2) the molecule is more strongly adsorbed by metal surfaces than similar halogen compounds which do not contain oxygen. The latter circumstance enhances the effect of small amounts of such compounds, because it is equivalent to an increase in concentration of the compound at the bearing surfaces.

45 Diphenyl ether is an example of a compound which may be directly halogenated, or specifically chlorinated, to form a preferred type of product. The chlorination may be carried out so as to produce a material which consists almost entirely of substitution products by the use of a chlorine carrier such as iron, iron chloride or aluminum chloride, and maintaining the temperature at 150° C. or higher. A product containing up to about 45% chlorine may be easily prepared in this way. This product is a complex mixture of 50 chlorine substitution products ranging from the monochlor- up to and including the hepta- or octachlor- diphenyl ethers. The product may be further refined by treating with solutions of alkalies, or solid alkalies or alkaline earth oxides, to remove free acid and decompose such small amounts of addition products as may be present. The resulting product is itself a good lubricant with a high film strength; and may also be used to improve the lubricating quality, increase the 55 film strength, and inhibit deterioration in use,

of mineral lubricating oil when added in relatively small proportions.

The chlorinated diphenyl ether, prepared as described above may be further refined by vacuum distillation. The higher boiling fractions (e. g., that boiling at 370° to 390° under atmospheric pressure) are extremely stable viscous liquids also having superior lubricating qualities and especially suitable as lubricants at high temperatures where high speeds are encountered (e. g., turbines operated with high pressure superheated steam). The vacuum-distilled product also is a valuable addition-agent for mineral lubricating oils and notably improves such oils for use as lubricants in internal combustion engines; e. g., in lubrication of cylinder walls, valves, valve stems, and crankshaft and connecting rod bearings.

It is especially valuable for use in such engines running at high speeds and under high loads, e. g., aircraft engines, Diesel engines, etc.

Diphenyl ether is also capable of forming chlorine addition products when chlorinated directly. The formation of such products is favored by:

- (1) Lower temperature (e. g. 100° C. or lower).
- (2) Absence of "chlorine carriers."
- (3) Chlorination by a counter-flow process, i. e., where the flow of liquid is in a direction counter to that of the gas flow in a single container; or where, in a multiple-container apparatus, the liquid is advanced toward the source of chlorine.

When chlorinated diphenyl ether is prepared so as to contain a substantial proportion of addition products (e. g., a mixture containing about 40% chlorine with about one-fourth of the chlorine in the form of addition products), it is desirable to remove the less stable material by treatment with an alkali. This is conveniently done by heating with crushed quick-lime to a temperature near the maximum temperature to be encountered by the material when in use. For example, for use as an addition to mineral oil to be used as a lubricant for slow-speed bearings, gears, etc. where very high unit pressures are encountered but the maximum temperature is low; the chlorinated diphenyl oxide containing chlorine addition products is advantageously treated with alkali at a temperature not to exceed, say, 50° C. For use in a lubricant for high speed gears, operating under high loads, the alkali treatment should be done at a higher temperature, say 100° C. The higher the proportion of addition products in the material, and the lower the temperature of alkali treatment, the more effective the resulting product as an "extreme pressure" lubricant, or addition agent for increasing the film strength of other lubricants. However, it is advisable to carry out the alkali treatment at a high enough temperature to insure stability in service.

The same principles apply to the halogenation of other analogous compounds, e. g., di-aryl ethers (specifically dixenyl ether, dinaphthyl ether, etc.) and aryl alkyl ethers, and to other aryl compounds, both oxygen-containing, and otherwise, e. g., naphthalene, anthracene, diphenyl; and their homologs, such as methyl and ethyl naphthalene, dibenzyl, ditolyl, etc.

When it is necessary or desirable, to use any halogenated material which contains an appreciable proportion of halogen in the form of unstable or easily hydrolyzed compounds, the corrosive effect of such unstable compounds offers a

serious objection. To overcome this corrosive effect, and actually improve the lubricating quality of the material, the same treatment as described above for the improvement of the chlorinated diphenyl ether containing addition products may be employed, i. e., treating with solutions of alkalies, or solid alkaline materials such as caustic soda or potash, sodium carbonate or bicarbonate, calcium oxide, hydroxide or carbonate, etc. When the halogen is in the form of an easily hydrolyzed compound, it is replaced by means of such treatment, with the hydroxyl radicle, thus improving the lubricating properties of the resulting product by the addition of combined oxygen.

Another type of treatment of such corrosive halogenated materials producing a greatly improved product for certain uses is to use hydro-sulphides, sulphides or polysulphides, etc. instead of oxides, hydroxides, carbonates, etc. In this case, the easily hydrolyzed halogen is replaced with sulphur or a sulphur-bearing radicle such as mercaptan.

These methods of treatment are particularly valuable for the preparation of improved lubricants from chlorinated complex materials, such as petroleum oils and products derived from them, animal and vegetable oils or any other commercial complex organic material which may be chlorinated.

Halogen bearing derivatives of certain of the compounds referred to above cannot easily be prepared by direct halogenation, and are preferably obtained in other ways. For example, tri-chlor-triphenyl-phosphate may be obtained by the reaction of phosphorus oxychloride with chlorphenol. Similar phosphates may be prepared in the same way from other chlorination products of phenol, cresols, xylenols, "tar acids," naphthols etc. From the same and similar chlorination products, derivatives of other acids may also be obtained. For example, those of the fatty acids may be prepared by reaction of the chlorinated phenol, or similar material, with the acid chloride, acid anhydride, or with the acid itself. Chlor phenol, or chlorphenyl phenol, for example, when heated with stearic acid will react to form chlorphenyl stearate, or chlorphenylphenyl stearate, respectively. Since it is difficult to carry the reaction with fatty acids to completion, a mixture of 50 to 60% of the reaction product together with the unreacted materials is conveniently prepared and is suitable for certain uses without further purification.

The presence of oxygen in the halogenated compound, if in relatively high proportion, has a tendency to lower the solubility of the product in mineral oil. This tendency may be overcome or offset, in four ways: (1) by hydrogenation; partial or complete, of the ring structure; (2) by the addition of alkyl radicles to the molecules containing the oxygen; (3) by complexity or molecular heterogeneity of the material used; and (4) by the addition of a liquid which will act as a mutual solvent, i. e., a liquid in which the solid material is soluble and which is completely miscible with mineral oil, for example, alkyl derivatives of naphthalene.

The effect of hydrogenation is illustrated by the relative solubilities in mineral oils of phenol and cyclohexanol, and of the corresponding chlorinated compounds. The effect of the addition of alkyl radicles is quite similar; cresol and the chlrcresols, for example, being more soluble than phenol and the corresponding chlor-phenols.

There are additional advantages in having a

complex mixture of more or less related compounds, because the resulting product, besides being more soluble in mineral oil, will be more easily handled and of a more suitable character for use as a lubricant by itself. This advantage is due to the fact that such mixtures have lower melting points and are usually relatively viscous liquids as compared with the pure components of the mixture. The complexity of the mixture may result from the multiplicity of compounds produced by chlorination of a single compound (e. g., as in the case of diphenyl ether, dixenyl ether, etc.) or may be still further enhanced by the use, as raw materials, of commercial products which are themselves of a complex nature, such as cresol, "tar acids," naphthenic acids, etc.

While it is preferable to have both oxygen and a halogen present in the same molecule, the results effected by the use of a halogen-bearing organic ring compound which does not contain oxygen may be improved by the addition of an organic oxygen compound. Such organic oxygen compounds may be any of the organic ring compounds listed above and in addition, any similar organic oxygen compounds which do not contain ring structures, e. g., alkyl, allyl, etc., alcohols, ethers, aldehydes, ketones, acids, esters and salts. Of these compounds the carboxylic acids and the esters and salts of such acids are preferred, e. g., fatty oils, vegetable oils, oleic acid, stearic acid, amyl acetate, butyl stearate, di-butyl phthalate, methyl salicylate, naphthenic acid, butyl naphthenate; sodium, calcium and aluminum stearates and oleates; sodium, calcium and lead naphthenates.

The above enumerated additions to lubricating oils for the purpose of increasing the lubricating properties thereof may, as previously indicated, be added to a pure hydrocarbon oil in order to improve its lubricating properties. Additionally improved results may be secured by the employment of these additions with an oil containing sulphur in some form.

The effect of sulphur and of sulphur compounds in increasing film strength is enormously enhanced by the presence of halogen- and oxygen-containing organic compounds, especially if the relative proportions of such sulphur and halogen compounds are within certain ranges. Sulphur compounds which have a negligible effect in increasing film strength by themselves are very effective when used in combination with the proper proportion of halogen- and oxygen-bearing organic compounds. Organic sulphides, disulphides, polysulphides, mercaptans, mercaptoles, thio-acids, dithioacids, sulphones, sulphoxides, sulphonic acids, sulphinic acids, sulphone amides, sulphone chlorides, thio-amides, thio-anilides, etc., (which may or may not contain a ring structure) are examples of sulphur compounds which act in this way. The table below shows the results obtained when solutions in mineral oil of such compounds, alone and with chlorinated diphenyl ether, were tested on an Almen lubricant testing machine. The chlorinated diphenyl ether contained a total of about 45% chlorine with about 10% chlorine in the form of addition products, and had been treated with quick-lime at a temperature of about 90° C. The increase in film strength of the oil caused by compounds dissolved in it is shown, and is stated in terms of additional pounds of weight applied to the loading arm of the machine required to cause breakdown, as compared with the oil alone.

|    | Percent of diphenyl sulphide              | Percent of chlorinated diphenyl ether | Increase in breakdown load |
|----|-------------------------------------------|---------------------------------------|----------------------------|
| 5  | 0                                         | 1                                     | 6                          |
|    | 0                                         | 2                                     | 8                          |
|    | 0                                         | 4                                     | 9                          |
|    | 5.8                                       | 0                                     | 2                          |
|    | 5.8                                       | 4                                     | 22                         |
| 10 | <i>Percent diphenyl disulphide</i>        |                                       |                            |
|    | 2                                         | 0                                     | 4                          |
|    | 2                                         | 1                                     | 22                         |
| 15 | <i>Percent dibenzyl disulphide</i>        |                                       |                            |
|    | 3                                         | 0                                     | 4                          |
|    | 3                                         | 1½                                    | +24                        |
| 20 | <i>Percent mercapto stearic acid</i>      |                                       |                            |
|    | 3                                         | 0                                     | 6                          |
|    | 3                                         | 1                                     | +24                        |
|    | <i>Percent di-methyl benzyl sulphide*</i> |                                       |                            |
|    | ½                                         | 0                                     | 3                          |
|    | ½                                         | 1½                                    | +24                        |

\*This material was an impure product containing about 10 per cent total sulphur and about 3 per cent total chlorine, the latter in non-hydrolyzable form. It was prepared by chlorinating boiling xylene until the boiling point reached 200° C. and allowing the chlorinated xylene to react with sodium sulphide in alcoholic solution. The product separated as a heavier oily layer and was treated with calcium oxide at 100° C.

30 Further improved results are obtained by the presence of a halogen in the compound containing the sulphur. For example, the sulphides, disulphides and polysulphides, of chlor-phenyl, chlor-benzyl, chlor-cresyl, chlor-xylyl, etc. give 35 improved results over the corresponding chlorine-free compounds. Still further improvement results from the introduction of oxygen into the same molecule with the sulphur, or with sulphur and chlorine. For example (1) dibenzoyl 40 dimethyl disulphide is more effective than the dibenzyl compound and the chlor-dibenzoyl compound still more effective, and (2) mercapto acids, such as mercapto stearic, are more effective than mercaptans, and chlor-phenyl mercapto stearate is still more effective.

45 Instead of sulphur compounds of the type described above, certain "sulphurized" compounds containing sulphur in more active or loosely combined form may be used. Examples of such materials are the products obtained by heating sulphur with certain mineral oils, or other petroleum derivatives, or with fixed oils (i. e., animal or vegetable oils), or sulphurized terpene (U. S. Patent No. 1,926,687) and other similar compounds. These materials are more or less effective when added to mineral oils by themselves, in increasing the film strength; but their effectiveness is greatly increased by the addition, with them, of a halogen and oxygen bearing organic 55 ring compound. An example is shown in the following data obtained on an Almen lubricant testing machine. The sulphurized cottonseed oil contained about 9½% of sulphur. As above, the results are stated in terms of additional pounds 60 of weight applied to the loading arm of the machine required to cause breakdown as compared with the oil alone.

|    | Percent of sulphurized cottonseed oil | Percent of chlorinated diphenyl ether | Increase in breakdown load |
|----|---------------------------------------|---------------------------------------|----------------------------|
| 70 | 0                                     | 1                                     | 6                          |
|    | 5                                     | 0                                     | 6                          |
|    | 5                                     | 1                                     | +24                        |

In order to protect bearings, gears, etc. from very severe overloads, it is sometimes advisable to use a halogen-containing compound which is so unstable as to be appreciably corrosive under normal conditions. Since chain compounds are generally more corrosive, i. e., more unstable than ring compounds, they are admirably suited for this purpose. In these circumstances the corrosive effect of such chain compounds and of halogenated organic ring compounds of the addition type for example, may be greatly inhibited by the addition of certain other oil-soluble compounds, such as (1) organic bases, aromatic and alkyl amines, triethanolamine, quinoline, etc., (2) organic phosphates, e. g. tri-butyl phosphate, 15 tri-phenyl phosphate, tri-cresyl phosphate, etc. Also certain of the halogen and sulphur compounds referred to above have similar corrosion-inhibiting effects, notably, (1) the phosphates of chlorinated ring compounds, e. g., tri-chlorphenyl phosphate, (2) mercaptans and chlor-mercaptans. 20

It has been found that suitable oil base containing from 0.10% to 2.50% of sulphur in free or combined form is best suited for use in a composition according to the present invention. These percentages are not to be construed, however, as limitations but merely as an indication of the range of sulphur in the form defined for optimum results. 25

30 Since generally the addition of certain of the halogen-bearing compounds of the class including the above enumerated reduce the viscosity of the oil base to which the same are added, if a large percentage of such compounds are added, there will be a tendency to destroy "thick-film" lubrication because of such reduction in viscosity. For ordinary use, if an excessive quantity of such compounds are added, all of the lubrication will then be of the "thin-film" type and therefore, 40 produce a decided increase in the amount of friction developed.

45 Optimum results are, therefore, obtained by using minimum quantities of those halogenated compounds which tend to reduce the viscosity of the oil base so that their beneficial effect in the region of "thin-film" lubrication will not be overshadowed by their detrimental effect in the region of "thick-film" lubrication.

50 Our invention contemplates incorporating with a suitable oil base a total of less than 20% of at least one halogenated oxygen-containing organic ring compound of those enumerated above. The above limit applied to the use of halogenated oxygen-containing organic ring compounds with 55 a suitable oil base for the purpose of producing a lubricating composition adapted for ordinary use. It is to be understood, however, and, as pointed out elsewhere herein, that certain of these compounds may be, for certain purposes and for 60 certain types of use, employed in a substantially pure state and as such, function in a very desirable manner as the only lubricant employed.

65 The optimum amount of the halogenated compound to be employed will depend largely upon the halogen content of the particular compound, its physical characteristics and especially its effect on the viscosity of the oil to which it is added. The particular use for which the lubricant is intended is also a governing factor in 70 determining the amount of the compound to be added.

75 For the purpose of lubricating and reducing the friction between the relatively movable parts of an internal combustion engine such as crank-

case bearings, piston and cylinder surfaces, as well as piston rings and valves, a composition according to our invention comprises a large proportion of a suitable oil base such as mineral oil and concentrations of from one-tenth to two per cent. of halogenated compounds of the above class containing from 50% to 25% of chlorine. If the valve structure of the engine is to be lubricated separately from the remainder of the mechanism or by means acting in an auxiliary fashion, the composition for such purposes will preferably contain a larger amount of such halogenated compounds, i. e., from 1 to 10%.

The limit of the amount of the halogenated compounds which may be added to an oily base and which will produce improved results largely depends, as above indicated, upon the reduction in viscosity of the composition caused by the addition of such compounds. Certain of the more viscous compounds, for example, chlorinated diphenyl ether containing about 50% chlorine, may be added in amounts exceeding 20% without causing too great a reduction of viscosity. For ordinary use the lubricating compositions embodying certain of the named addition agents may contain such agents up to 20% of the total composition.

When the halogenated compounds of the closed ring type, in contradistinction to the open chain type, are used, certain advantages are obtained which may be briefly explained as follows:

In case of oil in actual use in machinery of any kind and particularly in the crank case of internal combustion engines, moisture is always present to some extent and due to condensation, may even accumulate to form a separate layer. There is always sufficient water present, therefore, for hydrolysis to take place, particularly when the addition of a chlorinated compound is made to the extent of only a few per cent.

Experiments have shown that when compounds which readily hydrolyze, such as certain chlorinated open chain compounds, are added to the oily base, hydrolysis will take place to such an extent that the metal parts of any machine being lubricated will be seriously attacked and corroded by the acid generated. On the other hand, the addition of chlorinated carbon ring compounds of the above enumerated class does not cause corrosion.

The composition comprising our invention has certain advantages when used as a lubricant, of which the following may be mentioned—

First: By the use of this composition it is possible to extend the pressure range between the bearing surfaces because of the reduced tendency for bearing surfaces so lubricated to become scored or to seize at higher pressures than are allowable with ordinary lubricants.

Second: The friction between the bearing surfaces is reduced, especially in the higher pressure range, below that obtained with ordinary lubricants.

From the above description it will be noted that our invention comprises the combined use in a lubricating composition of oxygen and a halogen such as chlorine. It is also to be understood that while oxygen-bearing halogenated organic ring

compounds have been specifically referred to in this description as the combined source of the oxygen and chlorine, nevertheless, these two elements may be present in available form in separate compounds and preferably in separate organic compounds. As above pointed out, the organic ring compounds are preferred over the open chain compounds for the reason that the chlorine is sufficiently stable in the ring compounds so that in the presence of water there will be no appreciable amount of hydrolysis which would result in corrosion of the metal parts with which the composition comes in contact. In the form of the ring compounds the chlorine is sufficiently closely combined so that it will become available to chemically react with the bearing surfaces to produce the desired results only under the conditions imposed by the relative movement between such surfaces. In certain of the ring compounds, however, the chlorine is so closely attached that it is not made sufficiently available for the desired results even under the conditions imposed by the relative movement between the bearings. The additional presence of oxygen, however, cures this difficulty and it is this reason, among others, which may explain the unusual and unexpected results secured by the combined use in the composition of the oxygen and chlorine.

With regard to the use of sulphur-bearing oil in combination with halogenated compounds, it should be noted that for sufficiently desirable results, the major proportion of the ultimate composition need not consist entirely of sulphur-treated oil, but a suitable oil base such as mineral oil may have added thereto minor quantities or proportions of either a sulphur-treated oil or a sulphur compound, and a halogenated compound.

In the appended claims where sulphur is included in the composition, it is to be understood that such sulphur is in solution or in a stable form of colloidal suspension either in uncombined form or in the form of a sulphur compound.

This application is a division of application Ser. No. 737,070, filed July 26, 1934, and a continuation-in-part of co-pending applications Ser. Nos. 755,988, filed December 4, 1934, and 649,734, filed December 31, 1932.

Other modes of applying the principle of our invention may be employed instead of the one explained, change being made as regards the materials employed in carrying out the process, provided the ingredient or ingredients stated in any of the following claims or the equivalent of such stated ingredient or ingredients be employed.

We therefore particularly point out and distinctly claim as our invention:

1. A lubricating composition comprising a major proportion of mineral oil and minor proportions of both a halogenated organic compound and sulphurized mineral oil.

2. A lubricating composition which includes as a principal lubricating constituent the combination of a separate chlorinated organic compound and sulphurized mineral oil.

CARL F. PRUTTON  
ALBERT K. SMITH.